

W. A. SCOTT,  
ORE CONCENTRATION PROCESS,  
APPLICATION FILED AUG. 17, 1917.

1,246,665.

Patented Nov. 13, 1917.



Witness:

*C. Burnap*

Inventor:

*Walter A. Scott*

# UNITED STATES PATENT OFFICE

WALTER A. SCOTT, OF CHICAGO, ILLINOIS.

## ORE-CONCENTRATION PROCESS.

1,246,665.

Specification of Letters Patent.

Patented Nov. 13, 1917.

Application filed August 17, 1917. Serial No. 186,666.

To all whom it may concern:

Be it known that I, WALTER A. SCOTT, a citizen of the United States, residing at Chicago, in the county of Cook and State of Illinois, have invented certain new and useful Improvements in Ore-Concentration Processes, of which the following is a specification.

My invention is an improved flotation process. In the flotation process as previously practised, as is well known, certain reagents or modifying agents generally termed oils, although many of such substances are not oils, are added to a freely flowing ore pulp whereupon the introduction of air or some other gas into the pulp gives rise to the formation of bubbles which collect the desired mineral, generally metalliferous sulfids, and reject the gangue. The modifying agents used for this purpose comprise a great variety of oils, animal, vegetable and mineral oils, coal and wood tar and derivatives thereof, various alcohols, hydroxyl compounds and other substances, all of which I refer to herein, for the sake of brevity, as oils. Air, of course, is the most available gas and the one generally used, but in referring to air herein I include all gases which have a similar action.

Heretofore the air necessary in the operation of the process has been introduced into the ore pulp either by mechanical agitation which has the effect of beating in the air from the atmosphere, or by introducing air into the pulp through a porous medium forming part of the vessel in which the pulp is contained. Detailed explanation of the flotation process as heretofore practised is unnecessary in view of the fact that the process is widely known and described in many patents and publications, among them Patent No. 1,022,085 granted to J. M. Hyde April 2, 1912, Patent No. 1,104,755 granted to J. M. Callow July 29, 1914, and Patent No. 1,125,897 granted to J. M. Callow January 19, 1915.

In the operation described in the Hyde patent above referred to the air is beaten into the pulp by mechanical agitation, and in the operation described in the Callow patents above referred to the air is introduced under slight pressure through a porous medium, the pressure being just sufficient to over-balance the hydrostatic head of the pulp and to overcome the resistance of the porous medium. In the mechanical agita-

tion method of introducing air the mechanical agitation imparted to the pulp for that purpose is sufficient to thoroughly disseminate the oil through the pulp, such distribution of the oil being necessary in order that it may accomplish its function. In the method of introducing air through a porous medium it is necessary that independent means for mixing the oil be adopted and such independent means have heretofore taken the form of mechanical agitation sufficient to disseminate the oil, but not for the purpose of introducing air into the pulp and not having that effect to any appreciable or useful extent, reliance being placed for the introduction of air upon forcing it through the porous medium after the mechanical mixing of the oil with the pulp.

I have ascertained that the oil performs its principal, if not its only, function in the film surrounding the air bubbles and my invention consists in introducing the oil in such manner that it is supplied directly to the bubble films without the necessity of disseminating the oil through the entire body of ore pulp. My invention consists in using a volatile oil, impregnating the air with the gasified volatile oil, and introducing the gaseous mixture of air and oil into the pulp whereupon sufficient of the oil collects in the bubble films to effect the desired function. When operating according to my invention the necessity of mechanical agitation for the purpose of mixing the oil with the entire body of ore pulp is dispensed with and the amount of oil necessary for the purpose is greatly diminished in quantity by reason of the fact that the oil is applied directly to the bubble films where it is needed, without the necessity of distributing the oil throughout the body of the ore pulp in order to accomplish that purpose.

The drawing forming part of this application is a diagrammatic representation of means of applying my invention, and is a cross-sectional view of an apparatus designed for applying my invention by introducing the gaseous mixture of air and oil through a porous medium into the pulp.

In the figure A represents a containing vessel for the pulp, the same being provided with launders B into which the mineral bearing bubbles overflow. C represents the pulp contained in the vessel A and D the column of mineral bearing bubbles represented as filling the upper part of the ves-

sel A and overflowing into the launders B. E is a porous medium spaced some distance above the bottom of the vessel A, this porous medium being composed of several 5 layers of canvas or other fabric or of some other porous medium such as unglazed porcelain, or other substance. Between the porous medium E and the bottom of the vessel A there is an air space F into which air 10 under pressure is introduced through the pipe G. The air pressure in the space F is sufficient to support the head of pulp in the vessel A and to force the air through the pores of the medium E. H is a vessel containing some volatile oil and I represents a steam coil for heating the same, if necessary.

In operation the air supplied through the inlet pipe G becomes impregnated with gasified modifying agent which vaporizes 20 from the vessel H and the mixture of air and gasified oil penetrates the permeable medium E and rises as bubbles through the pulp C. The effect of this is to form the bubble column D above the pulp, the bubbles forming the bubble column having collected the metalliferous mineral during their passage through the pulp and subsequently being overflowed with the mineral into the launders B. The bubbles collected in the 25 launders B may be broken down by any suitable means, as by a spray of water and the precipitated mineral collected as concentrate. The concentrate so collected may, as customary, be retreated to further purify 30 it, if necessary.

While I have shown certain specific means for effecting the mixture of ore with gasified oil, it will be obvious that my invention is not restricted to the specific means shown, 40 nor is my invention restricted to the use of any particular volatile oil. A variety of suitable substances are volatile and many others such as coal tar, and the coal tar products contain volatile constituents.

45 What I claim is:

1. An ore concentration process comprising the operations of vaporizing a modifying agent and forming a mixture thereof with air, introducing said mixture through 50 a fine texture porous medium into an ore pulp and forming bubbles to which certain mineral particles in the ore adhere as said bubbles rise through the pulp, causing said mineral-bearing bubbles to form a column 55 of bubbles above the pulp and separating the mineral carried by the bubbles in the upper part of the bubble column from the remainder of the ore.

2. An ore concentration process comprising 60 the operations of vaporizing a modifying agent and forming a mixture thereof with air free from modifying agent in the liquid state, introducing said mixture into an ore pulp in the form of bubbles to which 65 certain mineral particles in the ore adhere

as said bubbles rise through the pulp, causing said mineral-bearing bubbles to form a column of bubbles above the pulp and separating the mineral carried by the bubbles in the upper part of the bubble column from 70 the remainder of the ore.

3. An ore concentration process comprising the operations of vaporizing a modifying agent and forming a mixture thereof with air free from modifying agent in the 75 liquid state, introducing said mixture through a porous medium into an ore pulp and forming bubbles to which certain mineral particles in the ore adhere as said bubbles rise through the pulp, causing said 80 mineral-bearing bubbles to form a column of bubbles above the pulp and separating the mineral carried by the bubbles in the upper part of the bubble column from the 85 remainder of the ore.

4. An ore concentration process comprising the operations of vaporizing a modifying agent and forming a liquid free mixture thereof with air, introducing said mixture into an ore pulp under pressure not substantially 90 greater than that necessary to sustain the hydrostatic head of the pulp, thus forming bubbles which are impelled upwardly through the pulp by their buoyancy only and to which certain mineral particles in 95 the ore adhere, causing said mineral-bearing bubbles to form a column of bubbles above the pulp, and separating the mineral carried by the bubbles in the upper part of the bubble column from the remainder of the 100 ore.

5. An ore concentration process comprising the operations of vaporizing a modifying agent and forming a mixture thereof with air, introducing said mixture through 105 a fine texture porous medium into an ore pulp under pressure not substantially greater than that necessary to sustain the hydrostatic head of the pulp and to overcome the resistance of the porous medium to 110 the passage of the gaseous mixture, thus forming bubbles which are impelled upwardly through the pulp by their buoyancy only and to which certain mineral particles in 115 the ore adhere, causing said mineral-bearing bubbles to form a column of bubbles above the pulp, and separating the mineral carried by the bubbles in the upper part of the bubble column from the remainder of the 120 ore.

6. An ore concentration process comprising the operations of exposing a body of liquid modifying agent having a relatively large exposed surface to a current of air thereby vaporizing part of said agent, introducing the mixture of air and vaporized modifying agent so formed free from any of such agent in liquid form into an ore pulp in the form of bubbles to which certain mineral particles in the ore adhere as 125 130

said bubbles rise through the pulp, causing said mineral-bearing bubbles to form a column of bubbles above the pulp and separating the mineral carried by the bubbles in 5 the upper part of the bubble column from the remainder of the ore.

7. An ore concentration process comprising the operations of exposing a relatively large surface of a liquid modifying agent

- 10 containing a volatile constituent to a current of air thereby vaporizing part of said agent, introducing the mixture of air and vaporized modifying agent so formed free from any of such agent in liquid form into an ore 15 pulp in the form of bubbles to which certain mineral particles in the ore adhere as said bubbles rise through the pulp, causing said mineral bearing bubbles to form a column of bubbles above the pulp and separating 20 the mineral carried by the bubbles in the upper part of the bubble column from the remainder of the ore.

8. An ore concentration process comprising the operations of exposing a relatively 25 large surface of heated liquid modifying agent to a current of air thereby vaporizing part of said agent, introducing the mixture of air and vaporized modifying agent so formed free from any of such agent in

liquid form into an ore pulp in the form of 30 bubbles to which certain mineral particles in the ore adhere as said bubbles rise through the pulp, causing said mineral bearing bubbles to form a column of bubbles above the pulp and separating the mineral 35 carried by the bubbles in the upper part of the bubble column from the remainder of the ore.

9. An ore concentration process comprising the operations of exposing a body of 40 heated liquid modifying agent having a relatively large exposed surface containing a volatile constituent to a current of air thereby vaporizing part of said agent, introducing the mixture of air and vaporized 45 modifying agent so formed free from any of such agent in liquid form into an ore pulp in the form of bubbles to which certain mineral particles in the ore adhere as said bubbles rise through the pulp, causing said 50 mineral bearing bubbles to form a column of bubbles above the pulp and separating the mineral carried by the bubbles in the upper part of the bubble column from the remainder of the ore.

In testimony whereof, I have subscribed my name.

WALTER A. SCOTT.